# EUROPEAN PATENT SPECIFICATION

(11) **EP 2 528 077 B1**
(45) Date of publication and mention of the grant of the patent: **06.04.2016**
(21) Application number: 11004375.9
(22) Date of filing: 27.05.2011
(51) Int. Cl.: C22C 27/06, H01H 11/04, H01H 1/02, H01H 33/664, C22C 9/00, B22F 1/00, B22F 1/02, C22C 1/04, H01H 33/662

(54) **Contact material for vacuum interrupter, and method of making a contact material**
Kontaktmaterial für Vakuumschalter und Verfahren zur Herstellung eines Kontaktmaterials
Matériau de contact pour interrupteur sous vide et procédé de fabrication d'un matériau de contact

(43) Date of publication of application: 28.11.2012
(73) Proprietor: ABB Technology AG, 8050 Zürich (CH)
(72) Inventor: Simon, Reinhard, Dr., 5405 Baden 5 Dättwil (CH); Gentsch, Dietmar, Dr.-Ing., 40882 Ratingen (DE)
(74) Representative: Schmidt, Karl Michael

(56) References cited:
- EP-A1- 1 528 581
- EP-A2- 0 903 760
- US-A1- 2002 144 977

## Description

### Background of the invention

The predominant contact materials for vacuum interrupters are Cu/Cr composite materials consisting of typically 50 - 75 wt.% copper and 25 - 60 wt.% chromium. Conventional powder metallurgy techniques are mainly used for the production of these materials. It is well known from experience that the chemical composition of the contact material is very important for the application in vacuum interrupters. E.g. interstitial gas contents as well as copper-oxides and chromium-oxides should be kept as low as possible. In addition it was empirically found, that the Cu/Cr material should contain the element Si in a small quantity < 1 wt.% (more preferable < 0.2 wt.%) in order to achieve a high short-circuit current interruption performance of the vacuum interrupter. Alumino- or silicothermic produced Cr powders are widely used as today's main raw powder sources for the production of Cu/Cr materials. The alumino- or silicothermic method (also known as Goldschmidt-Process) is a comparable cheap technique used in the chromium metal industry. In this process the metals Al or Si or a mixture thereof is used to reduce Cr₂O₃ to Cr via the following reactions:

Cr₂O₃ + 2 Al → 2 Cr (I) + Al₂O₃ (1)

2 Cr₂O₃ + 3 Si → 4 Cr (I) + 3 SiO₂ (2)

As a consequence of the reducing agents (Al or Si), Cr powder products contain residual contaminations of Si or/and Al in elemental and oxide form. The Cr is produced in batches in very big quantities (typical several tons each batch). In this rather rude technique a precise control of the Si contaminants is in practice impossible. As a consequence, there are rather high variations in local Si concentration within a production batch and of course from batch to batch. This is a severe problem for the vacuum interrupter application, where a very precise control of the Si content at ppm-level is needed. It was found experimentally that variations in Si content of the contact material, which are related to different chromium batches, can lead to a very poor and random current interruption performance.

In the EP 0 903 760 A2, as well as in the EP 1 528 581 A1 as well as in the US 2002/144977 A1 is disclosed a contact material with the features of the preamble of claim 1. Problem is, to introduce a Si concentration in a reproductive way.

So it is the object of the invention, to solve the above described problem in a way that enables a precise control of the Si concentration of Cu/Cr contact materials. Furthermore the Si is very homogeneously distributed within the contact material in order to generate the maximum doping effect. It results in a reliable performance of vacuum interrupters at very high level, which is independent of quality variations between different Cr raw powder batches.

### Description of the invention

The problems are solved with the invention in that way, that the chromium content above is above 10 wt.% and that the material is doped with silicon below 0,2 wt.% (2000 ppm Si) and the remainder is copper Cu, and that the microstructure consists of chromium (Cr) particles which are covered by a thin layer of silicon (Si) or Si-based material (e.g. SiOₓ).

Further advantageous is, that the silicon (Si) or Si-based material (e.g. SiOₓ) is located at phase boundaries between chromium (Cr) and copper (Cu) and is therefore homogeneously distributed within the microstructure.

In detail, the unnotched impact bending strength of the material is higher than 30 J/cm².

Furthermore the electrical conductivity of the material is in the range of 30-35 MS/m.

For realizing that in a process of making the same, the chromium (Cr) particles are coated with a silicon-precursor, in order to bring in the silicon.

To introduce the silicon in a very effective way, the silicon-precursor is preferably a polysilazane or similar Si-containing polymer.

It is mostly advantageous, to use a powder metallurgical process for making the contact material in that way, that the coated Cr particles are further mixed with copper, pressed into contact shape, and finally sintered.

An advantageous use of a material according to at least one of claims 1 to 5, made by a process according to at least one of claims 6 to 8, is, that the material is used for contacts or contact suface coverage material for low, medium or high voltage switchgears.
A further advantageous use of it is for shielding, or shielding surface coverage material for medium or high voltage switchgears, especially in implementation in vacuum interrupters for medium voltage.

The invention is displayed in its functionality in the following figure and the description of the figures.

The invented material consists of chromium (Cr) particles either dispersed or arranged in a network within a continuous copper (Cu) matrix phase. Alternatively chromium (Cr) and copper (Cu) can also form an interpenetrating network of phases, depending on the content of chromium (Cr) and copper (Cu). The Cr particles or Cr phases are covered by a silicon (Si) based coating. A schematic drawing of the microstructure is shown in Figure 1. Although the overall Si content in the Cu/Cr material can be low, a homogeneous distribution of the Si dopant within the material microstructure is present resulting from the distribution of coated Cr particles. Figur 1 shows the microstructure of the invented copper/chromium (Cu/Cr) contact material. A homogeneous doping with silicon (Si) is realized by coating of chromium (Cr) particles by a Si-precursor. Figure 2 therefore shows a SEM micrograph of a Si-doped (280 ppm) and sintered Cu/Cr material. The EDX linescan reveals Si at the Cr/Cr and Cr/Cu interfaces, which result from the coating of Cr particles by Si-precursor.

In Figure 2 a typical microstructure of Si-doped and sintered Cu/Cr contact material is given. The SEM micrograph reveals that Si is located as a coating on Cr particles. The Si can be clearly detected at Cr/Cr and Cr/Cu interfaces by a simple EDX linescan or any or any other appropriate technique. The Cr particles are well dispersed in the Cu matrix phase and in consequence the thin Si layers located at the Cr particle surfaces result in a homogeneous distribution of Si-dopant throughout the whole microstructure. It was found by the inventors that this kind of doping can affect the interface properties between Cr and Cu. The described Si-doped material exhibits an improved short-circuit current interruption as well as improved mechanical and electrical performance.

The problem of homogeneous distribution and precise control of Si dopant in Cu/Cr contact materials is solved by coating the Cr particles with a Si-precursor in a very simple wet-chemical process. In the described invention a polysilazane of the type PHPS (= perhydropolysilazane) was typically used as Si-precursor. In principle every type of polysilazane or other similar Si-containing precursor can be used to achieve the preferred Cu/Cr microstructure of the invented material. The coating causes a very homogeneous distribution of Si in the final Cu/Cr material, which is important to generate a maximum doping effect. Moreover by adjusting the Si-precursor concentration, a precise control of Si content of the final Cu/Cr material is easy to achieve. This guarantees a reliable performance of vacuum interrupters and a stable contact material production independent of raw powder variations.
The preferred PHPS precursor is purely inorganic. ( Figure 3a) No carbon is included in the polymer structure. PHPS is readily soluble in non-polar organic solvents, like dibutylether, giving a transparent solution of very low viscosity (similar to water). The solvent is easily removable in air by evaporation. As already mentioned in principle every polysilazane or Si-containing precursor could be used. Nevertheless, for clarity of the invention the preferred precursor is specified in this document.

For the coating of Cr powders diluted precursor solutions can be made. Dibutylether is used as a solvent. The PHPS concentration in the precursor solution is typically in the range of 0.5 - 1.5 wt.%. It can be easily adjusted to the target Si value of the final Cu/Cr material. By this a precise control of final Si-concentration in the ppm-range is achieved. For the coating process the Cr powder is simply immersed in the precursor solution. The precursor reacts immediately with the particle surface forming strong chemical (covalent) Si-O-Cr bonds. After a few minutes of mixing, the dibutylether is removed by evaporation. Most of the solvent is recovered in a condensation gap and can be reused. The resulting dry Cr powder particles are covered with a thin layer (few nm thick) of Si-precursor. Due to the fact that the drying step is performed in air, the Si-precursor layer on top of the Cr particle surface undergoes a slow cross-linking reaction which starts when the dried Cr powder comes in contact with air. The NH-groups of the PHPS react with moisture (H₂O) in the air to form Si-O-Si cross links and gaseous ammonia (see Figure 3b). The resulting coating on the Cr particles is transformed into a dense SiOₓ layer. The Cr powder can be immediately mixed with Cu powder and subsequently pressed and sintered to a dense Cu/Cr contact material. Alternatively the coated Cr powder can also be stored and mixed with Cu powder to a later stage in order to continue the conventional powder metallurgy process by pressing and sintering to the final Cu/Cr contact material.

In Figure 4 a SEM micrographs of the uncoated and coated Cr powder are presented. The coated powder exhibits a very homogeneous Si distribution covering all surface area of the Cr particles. The colour code red expresses Si in the EDX mapping. XPS measurements revealed that the PHPS precursor was transformed during a full cross-linking reaction to a dense SiOₓ layer, with x ranging from ~0.9 to ~1.1 on the outmost surface region (4 - 5 nm). After the full powder metallurgy processing to a sintered Cu/Cr contact material the Si concentration was measured by ICP-OES. The measured concentration of 280 ppm Si matched the target value of 290 ppm very well. (Figure 4b)

In the following, the main advantages of the invention are summarized briefly.
- Homogeneous and precisely controllable doping of Cu/Cr materials with Si forming a thin coating of Cr particles in the final microstructure.
- Homogeneous and precisely controllable doping of Cu/Cr materials with Si forming a thin coating of Cu particles in the final microstructure.
- Improvement of the current interruption performance of Cu/Cr contact materials and stable control of performance independent of variations in Cr raw powder quality.
- Improvement of the impact strength and fracture behaviour of Cu/Cr contact materials by strengthening of the Cu/Cr phase boundary.
- High electrical conductivity of the invented Si-doped contact material.

In order to demonstrate the fundamental different behaviors of undoped and Si-doped Cu/Cr contact materials, two typical examples for both types of material are given in the following. Both materials have been processed using the same raw powder source and almost identical processing steps. The only difference in processing was in the doping with Si. One was undoped (not coated with the Si precursor) and the other one was Si-doped (coated with the Si precursor). In order to evaluate the current interruption performance of contact materials, they are installed into commercial vacuum interrupters of the same design and tested under the same conditions. A standard three-phase electrical test procedure is performed to determine the limit in short-circuit current interruption ability.
In Figur 5 a graphical summary of the different observed interruption performance of undoped and Si-doped Cu/Cr materials is given. The red line in the graph marks the rated short circuit current of the used vacuum interrupter design. As can be seen, the undoped contact material is able to interrupter successfully the demanded value of 21 kA rms. However, interruption failure occurred at the next increased current step at 23.6 kA rms. The material offers no safety margin. In this case the interruption performance is very susceptible to small variations in Cr raw powder quality, which can lead to interruption failure already below the demanded rating.
In contrast, as can be seen clearly, the Si-doped material is able to interrupt much higher currents. A successful interruption at a current of 33.1 kA rms is observed. This is equal to a safety margin of 58% well above the demanded rating. This outstanding performance of Si-doped material qualities is based on their microstructure as shown in Figure 1 and Figure 2.

A further improvement of Cu/Cr contact materials is achieved with respect to their mechanical performance. Contacts for vacuum interrupters have to withstand comparable high mechanical impact loads, because of the fast opening and closing speeds at which the interrupter is operated in service. It was found that Cu/Cr materials with Si-doping exhibit typically higher impact strengths compared with undoped materials. To give an example, in Figure 6, the impact strengths of two Cu/Cr materials are compared. Both materials have been processed using the same raw powder source and almost identical processing steps. The only difference in processing was in the doping with Si. One was undoped (not coated with the Si precursor) and the other one was Si-doped (coated with the Si precursor). The doped material shows a significant increase in impact strength.
This difference in mechanical performance can be explained by the accompanying fracture surfaces. Figure 7 shows fractographs of both materials in direct comparison. In the case of an undoped material, rather large gaps between Cr particles and the surrounding Cu phase are visible (see arrows in pictures), which reveal a rather poor bonding between both phases. In contrast, the Si-doped material shows an improved bonding between Cr particles and the Cu phase. This in turn leads to a pronounced trans-crystalline fracture of Cr particles.

Figure 7 (a) shows the fracture surface of undoped Cu/Cr contact material shows large gaps between Cr particles and Cu matrix phase (see yellow arrows in pictures). The bonding between Cr and Cu phase is comparable poor. In Figure 7 (b) The Si-doped Cu/Cr contact material exhibits an improved interfacial bonding between Cr and Cu phases. Therefore, trans-crystalline fracture of Cr particles is frequently observed (see green arrows in pictures).

Another important material property for the application in vacuum interrupters is the electrical conductivity of the contacts. In their major applications vacuum interrupters are operated in closed position most of the lifetime. A high electrical conductivity is of significant advantage in order to generate minimum losses under nominal currents. It is therefore important to note, that Si-doped Cu/Cr materials offer a comparable high electrical conductivity. This result was surprising, as usually almost all additives to copper based conductor materials lead basically to a decrease in electrical conductivity. However, the electrical conductivity of Si-doped Cu/Cr material (containing 280 ppm Si) is even higher than of the same undoped Cu/Cr material. Tab 1 summarizes the electrical conductivities of both materials, which have been processed almost identical. The only difference was in the doping with Si.

### EXAMPLES

### Example 1

A chromium raw powder batch with a measured (by ICP) Si content of 88 ppm was used as starting material. The target value of Si concentration in the final Cu/Cr contact material was set to be 290 ppm. A concentrated solution of 20 wt.% PHPS precursor was further diluted to 1.00 wt.% PHPS by addition of dibutylether. 1000 g of chromium powder was added to 128.0 g of the diluted precursor solution and mixed for a short period (< 30 min). After this the dispersion is dried by removal of the dibutylether solvent by rotational evaporation at a pressure of 40 mbar and a temperature of 60°C for approximately 1 hour. After this treatment the dry Cr powder was mixed with Cu powder in the ratio 25 wt.% Cr to 75 wt.% Cu. After pressing the Cu/Cr powder mixture and final sintering to a dense contact material the Si content was determined (by ICP) to be 280 ppm. The Si is homogeneously distributed within the sintered microstructure. The Si is typically located at the phase boundary between Cr and Cu.

### Example 2

A chromium raw powder batch with a measured (by ICP) Si content of 52 ppm was used as starting material. The target value of Si concentration in the final Cu/Cr contact material was set to be 600 ppm. A concentrated solution of 20 wt.% PHPS precursor was further diluted to 1.40 wt.% PHPS by addition of dibutylether. 1000 g of chromium powder was added to 232.0 g of the diluted precursor solution and mixed for a short period (< 30 min). After this the dispersion is dried by removal of the dibutylether solvent by rotational evaporation at a pressure of 40 mbar and a temperature of 60°C for approximately 1.5 hours. After this treatment the dry Cr powder was mixed with Cu powder in the ratio 25 wt.% Cr to 75 wt.% Cu. After pressing the Cu/Cr powder mixture and final sintering to a dense contact material the Si content was determined (by ICP) to be 589 ppm. The Si is homogeneously distributed within the sintered microstructure. The Si is typically located at the phase boundary between Cr and Cu.

## Claims

1. Contact material for vacuum interrupter with copper Cu and chromium Cr as contents, wherein the chromium content is above 10 wt.% and that the material is doped with silicon below 0,2 wt.% (2000 ppm Si) and the remainder is copper Cu,
**characterized in**
**that** the microstructure consists of chromium (Cr) particles which are covered by a thin layer of silicon (Si) or Si-based material.

2. Contact material according to claim 1,
**characterized in**
**that** the microstructure consists of Copper (Cu) particles in fomr of Copper-powder, and the particles are covered with thin layers of Silicone (Si) or Si-based material.

3. Contact material according at least to claim 1, wherein the silicon (Si) or Si-based material is located at phase boundaries between chromium (Cr) and copper (Cu) and is therefore homogeneously distributed within the microstructure.

4. Contact material according at least to claim 1, wherein the Silicon or Si-based material is a mixture of coated Chromium and Copper powder.

5. Contact material according at least to claim 1, wherein the unnotched impact bending strength of the material is higher than 30 J/cm².

6. Contact material according at least to claim 1, wherein the electrical conductivity of the material is higher than 33 MS/m.

7. Contact material according at least to claim 1, wherein copper particles are coated with Si precursor.

8. Contact material according at least to claim 1, wherein both selected powders are coated with Si precursor.

9. Process for making the contact material according to one of claim 1 to 4, wherein chromium (Cr) particles are coated with a silicon-precursor.

10. Process for making the contact material according to claim 9, wherein the silicon-precursor is a polysilazane.

11. Process for making the contact material at least according to claim 7, or 8, or 9, or 10, **characterized in that** in a powder metallurgical process for making the contact material the coated Cr particles are further mixed with copper, pressed into contact shape, and finally sintered.

12. Use of a material according to at least one of claims 1 to 4, made by a process according to at least one of claims 9 to 11, **characterized in that** the material is used for contacts or contact suface coverage material for low, or medium or high voltage switchgears.

13. Use of a material according to at least one of claims 1 to 4, made by a process according to at least one of claims 9 to 11, **characterized in that** the material is used for shielding, or shielding surface coverage material for low, medium or high voltage switchgears.

14. Use of a material according to claim 13, **characterized in that** the material is implemented in vacuum interrupters for medium voltage.

## Patentansprüche

1. Kontaktmaterial für eine Vakuum-Schaltröhre mit Kupfer Cu und Chrom Cr als Gehalte, wobei der Chromgehalt über 10 Gew.-% liegt und dass das Material mit Silizium unter 0,2 Gew.-% (2000 ppm Si) dotiert ist und der Rest Kupfer Cu ist,
**dadurch gekennzeichnet,**
**dass** die Mikrostruktur aus Chrompartikeln (Cr) besteht, die von einer dünnen Schicht aus Silizium (Si) oder Si-basiertem Material bedeckt sind.

2. Kontaktmaterial nach Anspruch 1,
**dadurch gekennzeichnet,**
**dass** die Mikrostruktur aus Kupferpartikeln (Cu) in Form von Kupferpulver besteht und dass die Partikel mit dünnen Schichten aus Silizium (Si) oder Si-basiertem Material bedeckt sind.

3. Kontaktmaterial nach mindestens Anspruch 1, wobei das Silizium (Si) oder das Si-basierte Material sich an Phasengrenzen zwischen Chrom (Cr) und Kupfer (Cu) befindet und deshalb innerhalb der Mikrostruktur homogen verteilt ist.

4. Kontaktmaterial nach mindestens Anspruch 1, wobei das Silizium oder das Si-basierte Material eine Mischung aus beschichtetem Chrom und Kupferpulver ist.

5. Kontaktmaterial mindestens nach Anspruch 1, wobei die reine Schlagbiegefestigkeit des Materials über 30 J/cm² liegt.

6. Kontaktmaterial mindestens nach Anspruch 1, wobei die elektrische Leitfähigkeit des Materials über 33 MS/m liegt.

7. Kontaktmaterial mindestens nach Anspruch 1, wobei Kupferpartikel mit einem Si-Vorläufer beschichtet sind.

8. Kontaktmaterial mindestens nach Anspruch 1, wobei beide gewählten Pulver mit einem Si-Vorläufer beschichtet sind.

9. Prozess zum Herstellen des Kontaktmaterials nach einem von Anspruch 1 bis 4,
wobei Chrompartikel (Cr) mit einem Siliziumvorläufer beschichtet sind.

10. Prozess zum Herstellen des Kontaktmaterials nach Anspruch 9, wobei der Siliziumvorläufer Polysilazan ist.

11. Prozess zum Herstellen des Kontaktmaterials mindestens nach Anspruch 7 oder 8 oder 9 oder 10, **dadurch gekennzeichnet, dass** in einem pulvermetallurgischen Prozess zum Herstellen des Kontaktmaterials die beschichteten Cr-Partikel weiter mit Kupfer gemischt, in eine Kontaktform gepresst und schließlich gesintert werden.

12. Verwendung eines Materials nach mindestens einem von Ansprüchen 1 bis 4, hergestellt durch einen Prozess gemäß mindestens einem der Ansprüche 9 bis 11, **dadurch gekennzeichnet, dass** das Material für Kontaktoberflächen oder ein Kontaktoberflächenbedeckungsmaterial für Nieder- oder Mittel- oder Hochspannungsschaltanlagen verwendet wird.

13. Verwendung eines Materials nach mindestens einem der Ansprüche 1 bis 4, hergestellt durch einen Prozess gemäß mindestens einem der Ansprüche 9 bis 11, **dadurch gekennzeichnet, dass** das Material zur Abschirmung oder als Abschirmungsoberflächenbedeckungsmaterial für Nieder-, Mittel- oder Hochspannungsschaltanlagen verwendet wird.

14. Verwendung eines Materials nach Anspruch 13, **dadurch gekennzeichnet, dass** das Material in Vakuum-Schaltröhren für Mittelspannung implementiert wird.

## Revendications

1. Matériau de contact pour interrupteur sous vide avec du cuivre Cu et du chrome Cr comme constituants, la teneur en chrome étant supérieure à 10 % en poids et le matériau étant dopé avec du silicium à moins de 0,2 % en poids (2000 ppm Si), et le reste étant du cuivre Cu,
**caractérisé en ce que**
la microstructure est composée de particules de chrome (Cr) qui sont enrobées d'une couche mince de silicium (Si) ou de matériau à base de Si.

2. Matériau de contact selon la revendication 1,
**caractérisé en ce que**
la microstructure est composée de particules de cuivre (Cu) sous forme de poudre de cuivre, et les particules sont enrobées de couches minces de silicium (Si) ou de matériau à base de Si.

3. Matériau de contact selon au moins la revendication 1, dans lequel le silicium (Si) ou le matériau à base de Si est situé aux limites de phase entre le chrome (Cr) et le cuivre (Cu) et est par conséquent distribué de façon homogène à l'intérieur de la microstructure.

4. Matériau de contact selon au moins la revendication 1, dans lequel le silicium ou le matériau à base de Si est un mélange de poudre de chrome et de cuivre enrobée.

5. Matériau de contact selon au moins la revendication 1, la résistance à la flexion par choc sur barreau non entaillé du matériau étant supérieure à 30 J/cm².

6. Matériau de contact selon au moins la revendication 1, la conductivité électrique du matériau étant supérieure à 33 MS/m.

7. Matériau de contact selon au moins la revendication 1, dans lequel les particules de cuivre sont enrobées d'un précurseur de Si.

8. Matériau de contact selon au moins la revendication 1, dans lequel les deux poudres sélectionnées sont enrobées d'un précurseur de Si.

9. Procédé de fabrication du matériau de contact selon une des revendications 1 à 4, dans lequel des particules de chrome (Cr) sont enrobées avec un précurseur de silicium.

10. Procédé de fabrication du matériau de contact selon la revendication 9, dans lequel le précurseur de silicium est un polysilazane.

11. Procédé de fabrication du matériau de contact selon la revendication 7, ou 8, ou 9, ou 10, **caractérisé en ce que** dans un procédé de métallurgie des poudres pour la fabrication du matériau de contact les particules de Cr enrobées sont en outre mélangées avec du cuivre, comprimées en une forme compacte, et enfin frittées.

12. Utilisation d'un matériau selon au moins une des revendications 1 à 4, fabriqué par un procédé selon au moins une des revendications 9 à 11, **caractérisée en ce que** le matériau est utilisé pour des contacts ou un matériau de revêtement de surface de contact pour appareillages de commutation basse, ou moyenne, ou haute tension.

13. Utilisation d'un matériau selon au moins une des revendications 1 à 4, fabriqué par un procédé selon au moins une des revendications 9 à 11, **caractérisée en ce que** le matériau est utilisé pour un blindage, ou un matériau de revêtement de surface de blindage, pour appareillages de commutation basse, moyenne ou haute tension.

14. Utilisation d'un matériau selon la revendication 13, **caractérisée en ce que** le matériau est mis en oeuvre dans des interrupteurs sous vide pour moyenne tension.
